

1

3,696,078

### ANTISTATIC NYLON FILAMENTS

Andrew I. Smith and Roland J. Bryan, Jr., Pensacola, Fla., assignors to Monsanto Company, St. Louis, Mo.  
No Drawing. Filed Aug. 13, 1970, Ser. No. 63,664  
Int. Cl. C08g 20/38

U.S. Cl. 260—78 S

7 Claims

### ABSTRACT OF THE DISCLOSURE

The antistatic property of nylon filaments containing from about 2% to 15% by weight of a poly(alkylene ether, polyethoxylated hydrogenated castor oil, or polyethoxylated distearylamine dispersed therein) is greatly improved by also dispersing into the nylon from 0.5 to 5% by weight of a phosphonium bromide of the formula



where R' and each R are hydrocarbon radicals.

### BACKGROUND OF THE INVENTION

It is known that nylon yarns composed of filaments containing a polyethoxylated, hydrogenated castor oil or a high molecular weight polyethylene glycol dispersed therein as a separate phase are more conductive than regular nylon yarns and, as a result, have an improved antistatic property. We have found that the conductivity of the poly(alkylene ether)-containing nylon yarns can be further improved by rinsing the yarns after scourings or dyeing operations in various salt solutions such as aqueous solutions of sodium acetate, sodium chloride, etc. Such treatment is apparently effective because the salt solutions diffuse into the small pores of the yarns that are formed during the spinning process and from which a portion of the water-soluble polyethoxylated hydrogenated castor oil or polyethylene glycol is leached during the scouring or dyeing operations. However, this improved conductivity is either partially or completely lost when the treated yarns are either rinsed or further washed in non-salt-containing water, e.g., as by machine laundering.

The primary object of the present invention is to improve the antistatic properties of nylon filaments containing a poly(alkylene ether), polyethoxylated hydrogenated castor oil or polyethoxylated dialkylamine therein.

### SUMMARY OF THE INVENTION

The present invention provides nylon (polycarbonamide) filaments containing dispersed therein, in addition to a poly(alkylene ether, polyethoxylated hydrogenated castor oil or polyethoxylated distearylamine) from 0.5 to 5% and, preferably, 0.5 to 3% by weight, based

2

on the weight of the nylon, of a phosphonium bromide selected from the group consisting of



wherein each R is a monovalent, saturated hydrocarbon radical and R' is a divalent, saturated hydrocarbon radical. R' and each R generally contain from 1 to 12 carbon atoms, although each radical may contain more carbon atoms, if desired. Representative R radicals include methyl, ethyl, butyl, decyl, etc., phenyl, cyclohexyl, methyl-phenyl, benzyl, and the like. Representative R' radicals include xylylene (e.g. paraxylylene), C<sub>2</sub> to C<sub>12</sub> alkylene radicals, radicals of the structure



where m is 2 to 4, and of the structure



where p is 0 to 4, etc. The phosphonium bromides may be prepared by reacting a tertiary phosphine (R<sub>3</sub>P) with an organic bromide (RBr) or (R'Br).

Poly(alkylene ethers), polyethoxylated hydrogenated castor oils and polyethoxylated distearylamines which are useful in providing the nylon filaments of the present invention are those having a molecular weight of at least 1,000 (e.g. 1,000 to 30,000). The poly(alkylene ethers) have recurring —R''O— units wherein R'' is an alkylene radical having from 2 to 4 carbon atoms. The polyethoxylated distearylamines and polyethoxylated hydrogenated castor oils containing at least 70% by weight of recurring —CH<sub>2</sub>CH<sub>2</sub>O— units. These polyalkoxylated compounds may be formed by reacting an alcohol, hydrogenated castor oil or distearylamine with an appropriate amount of a C<sub>2</sub> to C<sub>4</sub> alkylene oxide, such as ethylene oxide. Representative poly(alkylene ethers) include: polyethylene glycol, polypropylene glycol, block copolymers of polyethylene glycol and polypropylene glycol, polyethoxylated lauryl alcohol and the like. Generally, from 2% to 15% by weight of the polyalkoxylated compound is incorporated into the nylon polymer.

The term nylon is used herein to denote linear, fiber-forming polycarbonamides which contain recurring carbonamide units separated from one another by at least



two carbon atoms. These polycarbonamides are well known in the art and are in general formed by heating an aqueous solution of a salt of a diamine and a dicarboxylic acid or by polymerization of a lactone. Representative polycarbonamides or nylons include polyhexamethylene adipamide (nylon 6,6), polyhexamethylene sebacamide (nylon 6,10), polyhexamethylene terephthalamide, polycaprolactam (nylon 6), etc.

The phosphonium bromides may be added to the nylon salt or salt solution prior to the evaporation or polymerization cycles, or during the polymerization cycles, or they may be stirred into the molten polymer during the holding (equilibrium) cycle when polymerization is essentially completed. Preferably, the phosphonium bromides are first mixed with one or more of the polyalkoxylated compounds described herein and then the resulting mixture or blend is stirred into the molten polymer during the holding cycle.

The phosphonium bromides by themselves do not improve the conductivity of nylon yarn. However, when the bromides are added to nylon in addition to one or more of the polyalkoxylated compounds described herein yarns made therefrom are more conductive than like yarns containing only said polyalkoxylated compound(s).

#### DESCRIPTION OF THE PREFERRED EMBODIMENTS

The following example is given to more fully illustrate the invention. In the example percentages and parts are by weight unless otherwise specified.

##### Example

Twelve yarns were prepared, each according to the following procedure:

To a stainless steel, high pressure autoclave was added 151 parts of hexamethylene ammonium adipate and 50 parts of water. The autoclave was equipped with stirring means to permit the contents to be agitated. The phosphonium bromide (and the amount thereof) indicated in the table was dissolved in water and added to the adipate salt solution. The autoclave was purged of oxygen by use of purified nitrogen and the temperature and pressure were slowly raised until values of 243° C. and 250 p.s.i.g. were reached. During this time steam was continuously removed from the autoclave as a condensate. The pressure was then gradually reduced to atmospheric over a 25 minute period. The polymer was then permitted to equilibrate for 30 minutes at 278° C., during which time an amount of a polyethoxylated compound, indicated in the table, was blended into the polymer melt by stirring at 244 r.p.m. for 25 minutes. The finished polymer was melt spun directly from the bottom of the autoclave through a 13-hole spinneret to yield white multifilament yarn. The yarn was drawn to provide a yarn having a denier of approximately 70 with a 35% elongation. Each of the twelve yarns was knitted into a tubular fabric and tested for static build-up.

In testing for static build-up each fabric was blank-dyed for one hour at the boil with a 40:1 liquor-to-goods ratio with 0.5% of sodium-N-methyl-N-oleoyl taurate. The fabric was rinsed for 15-20 seconds with deionized water (20:1 ratio) and then, after drawing for 30 seconds, was rinsed for 20 minutes with occasional stirring at a 40:1 ratio with deionized water. After drying for at least 16 hours at ambient conditions, the fabric was placed in a room with a Hayek-Chromey static instrument and permitted to equilibrate at 40% relative humidity for at least 2 days before static measurements were made. Then the tubular fabrics were folded lengthwise and placed in the Hayek-Chromey instrument sample holders. The instrument was run for one minute without contact between the sample fabric and the contact arm, which was covered with a finish-free nylon fabric, to determine the ground or starting charge (zero for all conducting yarns). The contact arm was then contacted with the rotating fabrics for 60 seconds to build up a static charge on the sample fabric. After the contact between the sample fabric and arm was broken, the time for half the accumulated charge on the sample fabric to dissipate therefrom was measured. The results of these tests are given in the table.

4  
TABLE

| 5            | Phosphonium type | Bromide amount, percent | Polyethoxylated compound |                 | Static half-life, seconds |
|--------------|------------------|-------------------------|--------------------------|-----------------|---------------------------|
|              |                  |                         | Type                     | Amount, percent |                           |
| Yarn sample: |                  |                         |                          |                 |                           |
| 1            |                  | 0 X                     |                          | 6.5             | 185                       |
| 2            | A                | 1 X                     |                          | 6.5             | 70                        |
| 3            | A                | 2 X                     |                          | 7               | 13                        |
| 4            | A                | 3 X                     |                          | 7               | 18                        |
| 5            | A                | 2 X                     |                          | 7               | 145, 14                   |
| 6            | A                | 2                       |                          | 0               | <sup>2</sup> >10          |
| 7            |                  | 0 Y                     |                          | 7               | 1484                      |
| 8            | A                | 2 Y                     |                          | 7               | 1153                      |
| 9            | B                | 3 0.4 X                 |                          | 7               | 12                        |
| 10           | C                | 1 X                     |                          | 7               | 63                        |
| 11           | C                | 3 0.4 X                 |                          | 7               | 32                        |
| 12           | B                | 1 X                     |                          | 7               | 71                        |

<sup>1</sup> Blank-dyed fabric heated 20 minutes at 150° C.

<sup>2</sup> Minutes.

<sup>3</sup> Added with poly(alkylene ether) during equilibrium cycle.

NOTE:

A=Methyltriphenyl phosphonium bromide

B=(n-Butyl) triphenyl phosphonium bromide

C=p-Xylylenebis(triphenyl phosphonium bromide)

X=Hydrogenated castor oil polyethoxylated with 200 moles of ethylene oxide per mole of oil having the structure:



Y=Polyethylene glycol (MW~20,000).

The phosphonium bromides (A, B and C) were purchased from Aldrich Chemical Co. and were used as received.

The results show that the addition of a phosphonium bromide per se to the nylon polymer did not improve the conductivity of the yarn, whereas the addition of both a phosphonium bromide and a polyalkoxylated compound of the type described herein to the nylon polymer rendered the yarn substantially more conductive than yarn containing only the said polyalkoxylated compound.

Similar results are also attained when other nylons, bromides and polyalkoxylated compounds of the type described herein are used instead of those specifically illustrated in the example.

We claim:

1. A static-resistant polycarbonamide filament containing dispersed therein (A) from 2 to 15% by weight of a compound having a molecular weight of at least 1,000, said compound being selected from the group consisting of poly(alkylene ethers) having recurring  $-\text{R}''\text{O}-$  units in which  $\text{R}''$  is a  $\text{C}_2$  to  $\text{C}_4$  alkylene radical, polyethoxylated distearylamine, polyethoxylated hydrogenated castor oil and mixtures thereof, wherein said polyethoxylated distearylamine and said polyethoxylated hydrogenated castor oil contain at least 70% by weight of recurring  $-\text{CH}_2\text{CH}_2\text{O}-$  units and (B) from 0.5 to 5% by weight of a phosphonium bromide selected from the group consisting of



wherein each R is a  $\text{C}_1$  to  $\text{C}_{12}$  monovalent hydrocarbon radical and R' is a  $\text{C}_6$  to  $\text{C}_{12}$  divalent hydrocarbon radical.

## 5

2. The filament of claim 1 wherein the said compound is polyethoxylated hydrogenated castor oil of the formula



in which the sum of  $x$ ,  $y$  and  $z$  equals an integer between 15 50 and 450.

3. The filament of claim 1 wherein the phosphonium bromide is a  $C_1$  to  $C_{12}$  alkyltriphenyl phosphonium bromide.

4. The filament of claim 1 wherein the phosphonium bromide is methyltriphenyl phosphonium bromide.

## 6

5. The filament of claim 1 wherein the phosphonium bromide is n-butyltriphenyl phosphonium bromide.

6. The filament of claim 1 wherein the phosphonium bromide is p-xylylenebis(triphenyl phosphonium bro-

mide).

7. The filament of claim 1 wherein the said compound is polyethylene glycol.

## References Cited

10

## UNITED STATES PATENTS

|           |         |         |       |          |
|-----------|---------|---------|-------|----------|
| 3,206,496 | 9/1965  | Rauhut  | ----- | 16—Dig.  |
| 3,226,178 | 12/1965 | Walker  | ----- | 17—Dig.  |
| 3,388,104 | 6/1968  | Crovatt | ----- | 260—78 S |
| 3,496,147 | 2/1970  | Cubbon  | ----- | 260—78 S |

HAROLD D. ANDERSON, Primary Examiner

U.S. Cl. X.R.

57—140 R; 260—18 N, 78 R, Dig. 16, 17, 19